

Nov. 24, 1936.

R. S. PULLEN

2,062,191

MATCH STRIKING COMPOSITION

Filed July 18, 1932

*Fig. 1.*



*Fig. 2.*



Fig. 3.



Inventor.  
Rodney S. Pullen.

Witnesses:

by C. Stull Johnson and Son  
Attorneys.

## UNITED STATES PATENT OFFICE

2,062,191

## MATCH-STRIKING COMPOSITION

Rodney Southwick Fullen, Akron, Ohio, assignor  
to Fullenlite Company, Philadelphia, Pa., a  
corporation of Pennsylvania

Application July 18, 1932, Serial No. 623,304

2 Claims. (Cl. 52—28)

My invention relates to the match-striking surfaces of safety matches of the type which ignite during withdrawal from the match packet.

By a match-striking surface I mean to designate the surface against which the head of the match is scratched in order to light the match. I wish to distinguish the match striking surface from the match head, which is not a part of my present invention and may be any match head suitable for use in a safety match.

10 A purpose of my invention is to form a match striking surface of markedly increased sensitivity for use with safety matches which ignite during withdrawal from the packet.

15 A further purpose is to improve the match striking qualities of water-proof striking surfaces used with safety matches of the pull-and-light variety by increasing the sensitivity of such striking surfaces.

20 A further purpose is to produce a composition for the match-striking surfaces of pull-and-light safety matches which will dry quickly, and therefore which is well adapted for machine application to the match packet.

25 A further purpose is to prevent destruction of the sensitiveness of the match-striking surface of a safety match due to "blushing" of the match-striking composition during its process of drying.

30 Further purposes will appear in the specification and in the claims.

My invention relates both to the methods involved and to the articles produced.

In the drawing I have illustrated one type only 35 of the many varieties of match packets to which my invention might be applied, choosing the form shown because it is conventional and largely typical of match packets of this type, and because it conveniently illustrates the principles of my invention.

40 I have also illustrated one form only of the many devices which might be used to prevent "blushing" of the striking material.

Figure 1 is a perspective view of a match packet 45 to which my invention has been applied.

Figure 2 is a top plan view of the blank from which the match packet of Figure 1 has been formed.

50 Figure 3 is a diagrammatic central vertical section of a heater for preventing "blushing" of my match-striking composition.

In the drawing like numerals refer to like parts.

The increasing prevalence of matches of the type which ignite during withdrawal from the 55 match packet (which I call for convenience "pull-

and-light" packets) has somewhat changed the requirements for match-striking compositions. Due to the danger of inadvertently igniting one or more matches, the matches of the pull-and-light variety are universally safety matches, and therefore they require a safety match striking surface.

However, the safety match striking surface in a pull-and-light packet must meet somewhat different conditions from those encountered by the striking surface on a box of safety matches, for example, or on a tear-off-and-strike packet of paper matches. In the pull-and-light packet, it is fundamental that the match can be drawn only once across the striking surface, and, therefore, the match head must be infallibly ignited in a single passage across the striking material.

Due to the weather conditions to which match packets are subjected, it is quite important that the match-striking surface be water-proof, so that it will not be injuriously affected by moisture. In seeking to develop a water-proof match-striking composition for use in a pull-and-light packet, I have found considerable difficulty in producing a material having the required sensitivity. Compositions which are in all respects satisfactory for use with box matches, for example, fail utterly to give satisfaction with pull-and-light matches because they are much too insensitive, and frequently fail to light a match during withdrawal.

I have discovered that the character of the solvent used in match-striking compositions is important in determining their suitability for my purpose.

As is common in striking compositions for safety matches, I employ red phosphorus as an essential ingredient. I add nitro-cellulose as a water-proofing material. As a solvent for nitro-cellulose, I find that it is quite important to use acetone rather than any other available solvent.

Acetone produces a match-striking surface of very high sensitivity, while other solvents, whose ability to dissolve nitro-cellulose is equal to or greater than that of acetone, fail to produce a sensitive striking surface.

Many solvents are entirely unsuited because of their excessive volatility, too great inflammability or very poisonous character. Ether is out of the question for all of these reasons.

The only solvent other than acetone whose properties compare favorably with those of acetone is amyl acetate, but it is distinctly inferior to acetone. Amyl acetate forms a lacquer-like film over the phosphorus after the match-strik-

ing composition dries, and this resinous coating appears to interfere with contact between the match head and the phosphorus of the match-striking material, thus decreasing the sensitivity of the match-striking material. Acetone, on the other hand, largely evaporates due to the fact that it is much more volatile than amyl acetate. As a consequence, when a match has been drawn across a striking surface prepared using acetone, the match will light infallibly, due, apparently, to the close contact possible between the phosphorus of the striking material and the match head. The abnormal and unexpected sensitivity of an acetone-dissolved match-striking surface has been proved repeatedly by my experiments.

The striking surface resulting from the use of acetone lacks considerable in toughness, so that it is unfitted for further use at a given locality after a match has been struck once at that place. 20 This characteristic entirely unfits an acetone dissolved striking surface for use on a box of safety matches, for example, where the same portion of the match-striking surface must be used repeatedly. However, the greatly increased sensitivity 25 of the acetone striking surface more than makes up for any possible disadvantage due to its tenderness, particularly where a given portion of the striking surface is used only once, as is true in a pull-and-light packet.

30 The striking surface resulting from the use of amyl acetate, on the other hand, is quite tough, but, due to its lack of sensitiveness, is unsuited for use on pull-and-light packets.

35 Acetone offers further practical advantages over amyl acetate as a solvent for nitro-cellulose. After drying, the composition produced by using acetone is practically odorless, but the composition formed with amyl acetate retains the strong odor of bananas or pears due to the amyl acetate 40 and this odor is very persistent and quite objectionable in a packet which must be carried in the pocket of the user.

During the application of the match-striking 45 composition to the match packet by machine, the use of amyl acetate as a solvent is particularly objectionable because of its slow-drying qualities. A composition in which acetone is employed as a solvent dries very quickly, on the other hand, therefore making possible increased speed of production.

50 My match-striking composition is preferably applied in the form of a paint. I do not concern myself in the present application with the particular method by which the match-striking composition is applied to the match packet. For example, it may be brushed on by machine or by hand, printed on or sprayed on.

In Figures 1 and 2 I show a conventional match 55 packet of the type in which the matches are ignited during withdrawal. The packet comprises a blank 20 having holes at 21 and 22 through which the matches 23 are threaded. The blank is scored at 24, 25, 26, 27, 28, 29 and 30, so that it may be folded as shown in Figure 1 into folded portions 31, 32, 33, 34, 35, 36, 37 and 38. The packet is held together in any suitable manner, as by a metallic clip 39.

On the portions 36 and 38 a match-striking 70 material is located at 40 and 41, made in accordance with my invention.

When the stick-end of a match 23 is pulled longitudinally of the match, the head passes through one of the holes 21 and then is rubbed 75 against the match-striking surfaces 40 and 41,

causing ignition. The head then passes through one of the holes 22.

I have secured very excellent results with a low percentage of red phosphorus, and in no case have I found it necessary to add more than 5% by weight of the total mixture. The remainder of the composition will comprise nitro-cellulose dissolved in acetone to the proper consistency, preferably that of paint.

I may obtain my nitro-cellulose from one of a number of sources. I preferably use the commercial product known as "cotton dope" but I may use some other form of nitro-cellulose or some material containing substantial quantities of nitro-cellulose, provided objectionable solvents are not present.

I may, if I desire, add abrasives, such as powdered glass, to my match-striking composition but I do not find that they are necessary.

In order to increase the adhesive qualities of 20 my match-striking composition, I may also add some glue, although this is not essential.

The proportions of the ingredients may vary somewhat according to the desired viscosity of the material when it is applied to the packet. I 25 preferably dissolve the nitro-cellulose in acetone, adding acetone until the composition is of about the viscosity of common paint, and introducing red phosphorus until it makes up say 5% of the mixture.

The red phosphorus is diffused uniformly 30 throughout the mixture, so that, after drying, some of it is available at the surface for ready contact with a match head.

I have found that my match-striking composition, 35 consisting of red phosphorus, nitro-cellulose and acetone, has a tendency to change its character during drying under certain weather conditions, particularly when the air is very moist. Under these conditions, the phosphorus settles to 40 the bottom of the striking film, injuriously affecting the sensitivity of the match-striking composition, and at the same time the composition becomes white in color. This change I call "blushing".

"Blushing" is not harmful, from the stand-point of change in color, but is particularly objectionable since it markedly decreases the sensitivity of the striking material. I find that I may avoid "blushing" entirely, where it exists, 50 by drying the match-striking material at elevated temperature. I find that a temperature of 175° F. will suffice to dry the match-striking material without the possibility of "blushing", although higher temperatures may be used.

As a convenient means of preventing "blushing", I pass the blank to which the match-striking material has been applied through a suitable drier. In Figure 3 I illustrate a drier 42 having a heating chamber 43 and heated in any suitable manner, as for example, an electrical resistance coil 44. A large blank 45, to which the match-striking material has been applied, is passed through the heating chamber 43 prior to cutting into small blanks 20.

It will be evident that additional ingredients of various sorts may be added to the red phosphorus, nitro-cellulose and acetone of my match-striking composition, without varying or destroying the effectiveness of the other ingredients.

In view of my invention and disclosure, variations and modifications to meet individual whim or particular need will doubtless become evident to others skilled in the art, to obtain all or part of the benefits of my invention without copying 70 75

the structure shown, and I, therefore, claim all such in so far as they fall within the reasonable spirit and scope of my invention.

Having thus described my invention, what I claim as new and desire to secure by Letters Patent is:—

1. The method of preventing injury to the sensitivity of a match-striking surface comprising red phosphorus, nitro-cellulose and acetone during drying of the surface which consists in

substantially increasing the temperature of the match-striking surface while it is drying, whereby "blushing" is prevented.

2. The method of preventing injury to the sensitivity of a match-striking surface comprising red phosphorus, nitro-cellulose and acetone during drying of the surface which consists in raising the surface to a temperature of above 175° F. during the drying period.

RODNEY SOUTHWICK PULLEN. 10